

Feb. 24, 1959

S. S. BERGH ET AL

2,875,104

SLAG-FORMING WELDING ELECTRODE

Filed May 16, 1955

Fig. 1. Fig. 2.



Inventors

Sven Sigvard Bergh  
Bölge Troberg  
Curt Anders Gustav Ericsson  
by Pierce, Scheffler & Parker  
attys

## SLAG-FORMING WELDING ELECTRODE

Sven Sigvard Bergh and Bolge Troberg, Vargon, and Curt Anders Gustav Ericsson, Surahammar, Sweden, assignors to Wargöns Aktiebolag, Vargon, Sweden, a Swedish company

Application May 16, 1955, Serial No. 508,766

Claims priority, application Sweden July 31, 1953

17 Claims. (Cl. 117—205)

This application is a continuation-in-part of our application Serial No. 380,862, filed September 17, 1953.

Slag forming welding electrodes are of two types, namely those having a core of iron or iron alloy with a slag forming coating and those having a shell or tube of iron or iron alloy filled with the slag forming material. In both cases metals and alloys in powdered form generally are included with the slag forming material. The purpose of such metal or metal alloy additions is to alloy with the core or shell metal and also to effect deoxidation. For this purpose both pure metals and metal alloys such as iron alloys e. g. ferromanganese and ferrosilicon for deoxidation and pure nickel, ferrochromium and ferromolybdenum for alloying have been used.

It has been shown that the commercial low carbon ferrochrome with a chromium content of 65—73% is very difficult to pulverize which makes the resulting powder relatively expensive and limits its use in welding electrodes.

The object of the present invention is to produce less expensive welding electrodes by the use of powder of iron alloy with a lower chromium content than the low carbon ferrochrome referred to above but not as low as that of the well known stainless and heat resisting iron-chromium steels.

Iron-chromium alloys, in the state of sigma phase, having a chromium content between about 30% and about 60% and the customary silicon and carbon contents have been found to be very brittle or capable of being made brittle. With pure iron-chromium alloys it generally is necessary to subject them to heat treatment to develop brittleness but brittleness can be developed also by additions of certain elements such as P, Si, Al, Mo, W, V, Ti, Zr, Cb, Ta, and Ni and Mn. These elements may be added in such substantial amounts that, without noteworthy loss of the brittle property, other alloying metals may be used such as Cu, Co and other metals, which per se are indifferent or which counteract the sigma phase formation. A high content of nickel or manganese counteracts the sigma phase formation. It is possible, however, to add nickel and manganese in high quantities provided that one or more of the aforesaid sigma promoting elements is present in a sufficient quantity.

According to the invention, said sigma phase formation is utilized in order to simplify the pulverization for manufacturing a powder to be used in welding electrodes and thereby lower the cost of the electrodes, and improve their quality. Some metals, e. g. nickel, cobalt and copper, are in pure form too soft to be ground into powder. When incorporated into a brittle sigma phase alloy, however, said soft metals may easily be ground together with the other elements contained in the alloy.

A phosphorus content of up to 1%, preferably 0.1% to 1%, a silicon content of up to 10%, preferably 1% to 10%, a molybdenum content of up to 10%, and a nickel content of 5% to 30% has been found suitable. It has been found that nickel may be replaced, wholly or partially, by manganese. Thus, e. g. in an alloy of the kind

referred to, one part by weight of nickel may be replaced by about two parts by weight of manganese, without noteworthy change of brittleness.

In case the alloy as originally produced is not sufficiently brittle, the desired brittleness can be imparted by a heat treatment at a temperature within the range 600—880° C.

As will be seen from the above, the brittle alloys, the powders of which are to be used in welding electrodes, depending upon their compositions, are either brittle as they are formed without any special embrittling treatment, or they are cooled from the liquid state under conditions designed to develop brittleness i. e. by cooling more or less slowly through the range from 880° C. to 600° C. or they are embrittled by being heated up for a sufficiently long time to within the range 600° C. to 880° C., preferably about 800° C. and then cooled. The brittle alloys are then pulverized and incorporated into the welding electrodes as cores or shells along with the slag forming materials in the customary way.

Welding electrodes of the two types referred to are illustrated in the accompanying drawings in which:

Fig. 1 is a longitudinal section of a welding electrode having a solid core and a slag-forming coating containing the sigma phase alloy, and

Fig. 2 is a longitudinal section of a welding electrode having a shell or tube of the welding metal and an inner slag-forming coating containing the sigma phase alloy.

When such an electrode is used, the brittle alloy powder contained in the shell will be remelted and simultaneously diluted with the core metal, e. g. iron or nickel, to such an extent that the brittleness disappears, i. e. the composition of the resulting alloy does not lie within the sigma phase range.

If the electrode consists of an iron or nickel tube and a slag forming core containing an alloy powder in the sigma form, the same thing will occur when the electrode is used.

Owing to the ternary, quaternary or still more complex composition of sigma alloy, its melting point is generally essentially lower compared to that of binary alloys. This is of very great importance when the alloy is used for the manufacture of welding electrodes and particularly when the electrode is to contain powders of metals melting at high temperature, e. g. tungsten. When using the electrode, the powder, the core material and possible fluxing agents are melted in the arc, and the melts are mixed in a short time, a low melting point being of the greatest importance.

By practicing the fundamental idea of the invention it is possible directly to manufacture uniform powders, which when used for welding electrodes of the types stated herein, combine in themselves the properties of previously added deoxidants, e. g. ferrosilicon and ferromanganese, and other alloying elements, mainly serving to be incorporated in the weld and to improve its properties in one way or another, e. g. for increasing the resistance to corrosion or erosion, increasing the refractory properties, improving the hardness, tenacity, or the like. These properties are obtained by suitably adapting the alloying elements in the powder, while considering the general rule that the composition shall be chosen so that a phase transformation can be obtained, which effects the brittleness. Thus, by suitably increasing the contents of silicon and manganese, it is possible to obtain a desired deoxidizing effect without loss of more expensive alloying elements. Further, by suitably adapting the nobler alloying ingredients, such as chromium, nickel, molybdenum, copper, cobalt, tungsten and carbide forming elements

such as titanium, vanadium, columbium, tantalum and zirconium, it is possible to obtain such a composition of the powder that when included in a welding electrode

with an unalloyed or alloyed core or case, on melting of the electrode there is produced a weld of corrosion-resistant or refractory properties and with a content of alloying elements which is at least as high as in the material, e. g. stainless steel, which is to be welded with said electrode, and consequently with at least as good properties as this material. If, according to these directions, there is to be manufactured a powder for use in electrodes with a low alloyed or unalloyed core, and the electrodes are to give a material in the weld of the so-called 18/8-type, i. e. a material containing about 18% chromium and 8% nickel and possibly also containing other metals which improve the properties, such as manganese, molybdenum, copper, aluminum, tungsten and carbide forming elements and others, the alloy from which the powder is manufactured according to the invention shall contain chromium and nickel and other alloying elements in such a ratio that the weld obtains the desired composition. When welding, there is usually a loss of chromium and, therefore, the ratio chromium to nickel should preferably be somewhat higher in the sigma alloy than what is desired in the weld.

As examples of compositions of alloys of the kind referred to herein which are brittle, the following may be cited.

Table

| Percent Cr | Percent Ni | Percent Mo | Percent Cu | Percent Al | Percent Si | Percent Ti | Percent Cb | Percent Co | Percent P |
|------------|------------|------------|------------|------------|------------|------------|------------|------------|-----------|
| 58         | ---        | ---        | ---        | ---        | 2.0        | ---        | ---        | ---        | ---       |
| 51         | ---        | ---        | ---        | ---        | 1.5        | ---        | ---        | ---        | ---       |
| 45         | 7          | ---        | ---        | ---        | ---        | ---        | ---        | ---        | ---       |
| 47         | 12         | ---        | ---        | ---        | 4          | ---        | ---        | ---        | 0.2       |
| 42         | 19         | ---        | ---        | ---        | ---        | ---        | ---        | ---        | ---       |
| 47         | 19         | ---        | ---        | ---        | ---        | ---        | ---        | ---        | ---       |
| 43         | 19         | 4          | 4          | ---        | ---        | 2          | 4          | ---        | ---       |
| 43         | 21         | 5          | 4          | ---        | ---        | 2          | 4          | ---        | ---       |
| 44         | 18         | 6          | 8          | ---        | ---        | 5          | ---        | 12         | ---       |
| 45         | ---        | ---        | ---        | 12         | 8          | 5          | ---        | 45         | ---       |
| 35         | ---        | ---        | ---        | ---        | ---        | ---        | ---        | ---        | ---       |

The rest in each case consists of iron with the accessory elements or impurities usually contained therein.

As a rule it can be said that the necessity for heat treatment decreases with increasing contents of elements such as silicon, molybdenum, tungsten, titanium and vanadium.

The invention is not limited with respect to the nature of the slag forming ingredient or the binder when the alloy powder is used in a welding electrode coating. The coating may be acid, neutral or basic.

We claim:

1. A welding electrode consisting essentially of a rod consisting principally of a metal selected from the group consisting of iron and nickel and a slag forming coating thereon, said coating containing a brittle sigma phase iron-chromium alloy having a chromium content of 30-60%, the ingredients of the coating and the rod being capable of forming an alloy which does not contain sigma phase when the electrode is used for welding.

2. Electrode as defined in claim 1, in which the iron-chromium alloy also contains nickel in quantity amounting to from 5% to 30%.

3. Electrode as defined in claim 2, in which at least

part of the nickel content is replaced by manganese, 1% of manganese replacing about 0.5% of nickel.

4. Electrode as defined in claim 1, in which the iron-chromium alloy also contains molybdenum in quantity up to 10%.

5. Electrode as defined in claim 1, in which the iron-chromium alloy also contains silicon in quantity up to 10%.

6. Electrode as defined in claim 1, in which the iron-chromium alloy also contains phosphorus in quantity up to 1%.

7. Electrode as defined in claim 1, in which the iron-chromium alloy consists essentially of 58% of chromium, 2.0% of silicon and 40% of iron.

8. Electrode as defined in claim 1, in which the iron-chromium alloy consists essentially of 51% of chromium, 1.5% of silicon and 47.5% of iron.

9. Electrode as defined in claim 1, in which the iron-chromium alloy consists essentially of 45% of chromium, 7% of nickel and 48% of iron.

10. Electrode as defined in claim 1, in which the iron-chromium alloy consists essentially of 47% of chromium, 12% of nickel and 41% of iron.

11. Electrode as defined in claim 1, in which the iron-chromium alloy consists essentially of 42% of chromium, 19% of nickel, 4% of silicon, 0.2% of phosphorus and 34.8% of iron.

12. Electrode as defined in claim 1, in which the iron-chromium alloy consists essentially of 47% of chromium, 19% of nickel, 4% of molybdenum and 30% of iron.

13. Electrode as defined in claim 1, in which the iron-chromium alloy consists essentially of 43% of chromium, 19% of nickel, 5% of molybdenum, 4% of copper and 29% of iron.

14. Electrode as defined in claim 1, in which the iron-chromium alloy consists essentially of 43% of chromium, 21% of nickel, 2% of titanium, 4% of columbium and 30% of iron.

15. Electrode as defined in claim 1, in which the iron-chromium alloy consists essentially of 44% chromium, 18% of nickel, 6% of molybdenum, 8% of copper and 24% of iron.

16. Electrode as defined in claim 1, in which the iron-chromium alloy consists essentially of 45% of chromium, 12% aluminium, 8% of silicon, 12% of cobalt and 23% of iron.

17. Electrode as defined in claim 1, in which the iron-chromium alloy consists essentially of 35% of chromium, 5% of titanium, 45% of cobalt and 15% of iron.

#### References Cited in the file of this patent

#### UNITED STATES PATENTS

|           |                   |               |
|-----------|-------------------|---------------|
| 1,241,899 | Armstrong         | Oct. 2, 1917  |
| 1,559,015 | Stoody            | Oct. 27, 1925 |
| 1,999,888 | Ammann            | Apr. 30, 1935 |
| 2,016,585 | Basore et al.     | Oct. 8, 1935  |
| 2,219,462 | Wissler           | Oct. 29, 1940 |
| 2,280,223 | Dumpelmann et al. | Apr. 21, 1942 |
| 2,291,482 | McLott            | July 28, 1942 |
| 2,299,483 | Lubbe et al.      | Oct. 20, 1942 |
| 2,408,620 | Friedlander       | Oct. 1, 1942  |